

## UNITED STATES PATENT OFFICE

2,440,837

## METAL CLEANING COMPOSITION

Hugh G. Webster, Detroit, Mich., assignor to  
J. H. ShoemakerNo Drawing, Application July 28, 1943,  
Serial No. 496,507

1 Claim. (Cl. 252—135)

1

This invention relates to a new composition of matter and to a process for utilizing it in aqueous solution for removal of oxides from metals which have been treated in a molten salt bath comprising sodium hydroxide, sodium nitrate, and preferably containing a small amount of sodium chloride.

In my joint application Serial No. 431,168, filed February 16, 1942 (now abandoned), there is disclosed the use of a molten salt bath comprising an alkali metal hydroxide, an alkali metal nitrate, and preferably a small amount of an alkali metal chloride for cleaning of metal surfaces, and particularly ferrous metal surfaces. The process comprises immersing the metal article in the molten salt bath of the above-mentioned composition, followed by an immersion in a dilute mineral acid such as hydrochloric or sulfuric acid. In the first step of the process, which is immersion in the molten salt bath, organic impurities on the metal surface are oxidized and therefore removed, and the inorganic impurities, such as graphite, carbon, and compounds of sulphur, silicon, phosphorus, etc. are converted into compounds which are readily removed from the metal surface in the dilute acid treatment. Treatment in the aqueous acid solution removes all the impurities from the surface of the metal and renders the metal surface clean and bright.

In my application Serial No. 473,397, filed January 23, 1943, I have disclosed a process for coating metal surfaces with protective lead alloys by immersion of the article in a molten salt bath described above, followed up by treatment in a dilute mineral acid, washing of the dilute mineral acid from the surface of the metal, and finally coating the metal surface with a protective lead alloy. The salt bath and acid treatments together convert the exposed surfaces of the metal pieces into etched matrices having minute foramina or pockets materially depleted of oxidized and non-metal substances. The etched matrices thus obtained have been found to form an exceedingly strong bond with high lead alloys when the alloy is suitably applied thereto.

In my joint application Serial No. 483,121, filed April 10, 1943 (now abandoned), is disclosed a new type of bearing and a process for preparing the new type of bearing in which a combination of molten salt and acid treatment is used to prepare a bearing back to receive a bearing alloy.

In all of these processes it is necessary to treat the surface of metal which has been immersed in the molten salt bath in an aqueous acid solution. This treatment in acid solution is not entirely

2

satisfactory. In spite of careful washing, there is a tendency for some acid to be retained on the surface of the metal. This acid has a deleterious effect on subsequent metal coating treatments.

- 5 It appears that even a brief immersion in dilute acid results not only in a removal of the oxide layer formed on the metal surface by the molten salt bath, but that some of the carbon and graphite in the metal just below the surface is exposed, causing the surface to be smudgy. Such a surface is unsuitable for coating operations. Furthermore, it has been found on certain types of ferrous metal articles that even a brief treatment in a dilute mineral acid results in strong adsorption of hydrogen on the surface of the metal. Hydrogen adsorption results in hydrogen embrittlement of the metal article, and thus for these types of ferrous metal articles the process is not applicable. The hydrogen adsorption tends to weaken the bond between the metal and the coating alloy. Also, when the process is used for preparing bearings, the hydrogen adsorption on the bearing back results in a weak bond between the bearing metal alloy and the bearing back. In the case of treatment of cast iron metal articles, it has been found that fairly prolonged treatment in the dilute acid is necessary to remove all of the oxide coating, and this pickling procedure has proved undesirable.
- 10 30 It is an object, therefore, of this invention to provide a process for preparing the surface of metals for coating operations by use of molten salts without use of acid solutions to remove the oxide layer formed in the molten salt bath.

- 35 Another object is to provide a process for cleaning metal articles by treatment in a molten salt bath comprising sodium hydroxide, sodium nitrate, and preferably containing a small amount of sodium chloride without the subsequent use of dilute mineral acids.

- 40 Another object of my invention is to provide a process for coating metal articles in which the metal article is prepared to receive the metal coating by treatment in a molten salt bath including an alkali metal hydroxide and nitrate without the use of acid solutions to remove the oxides from the surface of the metals after immersion in the molten salt bath.

- 45 Another object is a new composition of matter suitable when dissolved in water for removal of oxides formed on metal articles which have been immersed in a molten salt bath comprising an alkali metal hydroxide, an alkali metal nitrate, and preferably a small amount of an alkali metal chloride.

Still another object of my invention is a process for avoiding the use of acid solutions in the preparation of bearings by a process in which the bearing base is first immersed in a molten salt bath, followed by immersion in a molten metal bath for providing the bearing base with a high lead tinning alloy.

My invention has for further objects such additional operative advantages and improvements as may be found hereinbelow.

I have found that I may avoid the use of dilute acid to remove the oxide layers from metal articles immersed in molten salt baths if the acid solution is replaced by an aqueous solution of a composition comprising sodium hydroxide, sodium borate, sodium cyanide, and in some cases a small amount of either sulfur or sodium chloride, or both. This composition serves the same purpose as the dilute acids for removing the oxides and oxidized substances from the surface of the metal, but it has the advantage that the solution is alkaline and thereby any possibility of hydrogen adsorption or acid retention on the surfaces of metals is completely avoided.

In general the composition may vary over fairly wide limits. The sodium hydroxide may range from about 50 to about 90 parts, sodium borate from about 4 to about 10 parts, sodium cyanide from 5 to 46 parts, sulfur from .10 to about 4 parts, and sodium chloride from .10 to about 4 parts. The sodium hydroxide, sodium borate, and sodium cyanide are necessary components of the mixture, but the composition will operate without the use of sulfur or sodium chloride. However, the presence of either of these two substances, and preferably both of them, appears to have a beneficial action on the composition.

One composition which has been found to be particularly advantageous contains 70 parts sodium hydroxide, 18 parts sodium cyanide, 4 parts powdered borax, 4 parts sulfur, and 4 parts sodium chloride. This composition has been used to treat a wide variety of metal articles such as cast iron, spring steel, stainless steel, and other common ferrous metal alloys with good success. It has also been used with bronze, brass, and like alloys successfully.

While I have particularly described the sodium compounds, it will be obvious to those skilled in the art that any of the other alkali metal salts, such as potassium or lithium salts, may be used in making up the composition.

In practice, the composition is dissolved in water in a concentration about 8 pounds per gallon of water and heated to a temperature of about 220-250 degrees F., but of course below the boiling point of the solution. After the metal articles have been immersed in the molten salt bath and have been rinsed with wash water, they are immersed in this aqueous solution for a period of time sufficient to remove the oxide layer formed in the molten salt bath. The period of immersion will vary over wide limits and will depend to a considerable extent upon the condition of the metal surfaces and the type of metal being treated. In general, however, a period of 15 minutes has been found to be satisfactory in the usual type of articles. In the case of the treatment of bearings to prepare them to receive a tinning alloy, a period of 20 minutes has been found satisfactory for the average type of small bearings.

It appears that this composition has a dissolving action on the metal oxides and other oxidized substances on the surface of the metals. It is alkaline and has a reducing action to aid in

dissolving these substances from the metal surface.

By way of specific example of my invention, various metal articles, particularly susceptible to hydrogen embrittlement, have been treated in a solution containing one part by weight sodium nitrate, two parts by weight sodium hydroxide, and about .25 part by weight sodium chloride, and held in this bath for about 15 minutes at approximately 300 degrees F. When removed and rinsed, the surfaces of the metal parts exhibited a dull, dark finish. The metal parts were then immersed in an aqueous bath containing 70 parts sodium hydroxide, 18 parts sodium cyanide, 4 parts powdered borax, 4 parts sulfur, and 4 parts sodium chloride, made up to about 1.5 specific gravity and heated to 250 degrees F., and were maintained in this bath for about 15 minutes. After this treatment, the oxide layer was removed, and the articles had a metallic appearance, appearing to be clean of all surface impurities. All oxidizable substances, including carbon and graphite and compounds of sulfur, silicon, phosphorus, etc. were removed from the surfaces of the metals. These parts were then dipped in a molten lead alloy containing about 90 per cent lead, 5 per cent tin, and 5 per cent antimony. The lead alloy made a particularly firm bond on these articles, and were satisfactory in all respects, being free of pin holes, and having a uniformly coated surface. The articles showed no evidence of hydrogen embrittlement as would have been found if an acid treatment had been used to remove the oxide layer.

In another specific example of my invention I applied my process to certain cast iron parts. These parts presented a difficult problem as their surfaces held a considerable amount of adherent or imbedded silica. The parts were first immersed for five minutes in the molten salt bath of the same composition as that used in the preceding example. They were then removed, rinsed, and immersed in an aqueous solution of the same composition described in the preceding example, and maintained at about 270 degrees F. for about 20 minutes. Finally, they were taken out, rinsed, and dried, and were found to be particularly clean and suitable for coating operations. After dipping the parts in a molten lead alloy containing about 90 per cent lead, about 5 per cent tin, and about 5 per cent antimony, they acquired a uniform lead alloy surface free of pin holes and having no rivulets or dewetting. The bond between the coating lead alloy and the cast iron was particularly firm.

In still another example of my invention, a cast iron bearing back was subjected to the same treatment noted in the previous example. After the lead alloy surface had been put on the bearing back, the base was coated with a bearing metal containing about 1 per cent tin, 1 per cent arsenic, 15 per cent antimony, and the remainder lead, by pouring the molten bearing alloy on the bearing base to the desired thickness. This bearing was very satisfactory and had a very high shear strength. After the bearing was poured and solidified, it was annealed according to the ordinary practice. The bearing prepared in this fashion withstood the annealing operation without loosening of the bearing alloy from the back, whereas samples prepared in accordance with previous methods were not at all satisfactory when subjected to this test.

The use of this composition in connection with the molten salt bath treatment has several ad-

vantages. Because it is alkaline there can be no hydrogen adsorption on the surface of the metals, and therefore no hydrogen embrittlement and no deleterious action through retention of a small amount of acid on the surface of the metal. Furthermore, the composition has no tendency to attack the metal itself and therefore it does not expose additional graphite, carbon, or other impurities which are in the metals themselves but beneath the surface of the metal. Its only action is a reducing action in removing the metal oxides and other oxidizable substances from the surface of the metal.

While I have described my invention hereinabove with respect to particular applications and compositions and noting specific examples of alloys, it will be obvious to those who are skilled in the art that the invention is not limited to the specific examples of practice, but may be variously practised and employed within the scope of the claim hereinafter made.

What I claim is:

A metal cleaner comprising an aqueous solu-

tion of an alkali metal hydroxide, an alkali metal borate, and an alkali metal cyanide, in proportions, by weight, of 50-90 parts, 4-10 parts, and 5-46 parts, respectively.

HUGH G. WEBSTER.

#### REFERENCES CITED

The following references are of record in the file of this patent:

#### UNITED STATES PATENTS

| Number    | Name           | Date          |
|-----------|----------------|---------------|
| 838,810   | Roome          | Dec. 18, 1906 |
| 2,237,434 | Holden et al.  | Apr. 8, 1941  |
| 2,284,743 | Kawecki et al. | June 2, 1942  |
| 2,349,596 | Muskat         | May 23, 1944  |
| 2,380,284 | Young          | July 10, 1945 |

#### FOREIGN PATENTS

| Number | Country       | Date |
|--------|---------------|------|
| 10,177 | Great Britain | 1901 |